

## UNITED STATES PATENT OFFICE.

ROBERT MEZGER, OF STUTTGART, GERMANY, ASSIGNOR TO PAUL LECHLER, OF STUTTGART, GERMANY, A FIRM.

## SEALING MATERIAL FOR GASOMETERS.

No Drawing. Application filed November 21, 1925, Serial No. 70,710, and in Germany December 8, 1924.

My invention refers to a new product for use in sealing the gap between a dry gasometer casing and the disc movable therein, such gasometers being frequently used to 5 replace the old type of water-sealed gasometers. It is an object of my invention to provide means whereby the movable disc is packed in a gas-tight manner without its movability within the casing being impaired 10 and without danger of the substance used for packing or sealing being affected by the gas and by other causes.

In gasometers of the type aforesaid as hitherto in use the gap between the movable 15 disc and the outer casing is sealed as a rule by means of high temperature coal tar and the products of distillation obtained therefrom. It is generally inexpensive to use these substances inasmuch as this tar is 20 obtained as a by-product in the manufacture of illuminating gas.

It has, however, been shown that these products, if used for sealing purposes offer a number of material disadvantages. The 25 high temperature coal tar is known to thicken rapidly, partly by polymerization and partly by its lighter and even some of its more difficultly volatile constituents being carried away by the gas stored in the gasometer. In consequence of such thickening 30 of the tar the power required by the pumps serving to force the tar into the gap between the disc and the wall of the casing is unduly increased. The pumps being electrically connected and operated in an automatic manner are frequently affected by the thickening of the tar inasmuch as the overloading arising in consequence of such thickening causes the fuses to burn out. However, if the attendant fails to notice this, 40 the pumps will not work for a longer time and in consequence thereof the sealing will suffer so that comparatively great losses of gas may result. Moreover the most valuable parts of the tar are lost, the gas being at the same time carburetted, and these parts must be replaced, whereby the costs of operating a gasometer are unduly increased. A 45 thickened tar further has a higher freezing point as compared with the thinly fluid tar initially used and in consequence of this raising of the freezing point the operation 50

of a gasometer can be disturbed in winter unless sufficient heating is provided at all points where there is danger of freezing. 55 It has also been noticed that the water precipitated from the gas, such as water-gas, when cooling down, combines with the tar to form an emulsion and can be separated again from the tar only with great difficulty and only in very large gasometers, 60 such emulsions being so stable that for instance, even after an operation of four months the percentage of water in the tar has been found to be not less than twenty 65 percent. Obviously a high content of water will tend to further raise the freezing point of the tar, but the most dangerous consequence is the formation of ice on the inner walls of the gasometer which renders a tight 70 sealing impossible and forms a further source of danger. It is also evident that emulsions of this character will give rise to corrosion of the gasometer walls.

As is well known to any expert, a tar in 75 order to be fit for use as a sealing means for gasometers, must not suffer any perceptible change of boiling point curve and freezing point, if air is caused to pass through it for 6 hours at a temperature of 80 60° C. On being vigorously shaken with water in a separating funnel a clear separation of the water from the tar must be obtained after a short rest. I have now ascertained that all draw-backs are easily obviated if the high temperature coal tar and the products resulting therefrom are replaced by a solution of mineral bitumen in a mineral oil, brown coal tar oil or an oil obtained by distillation of low temperature 90 coal tar. I prefer using as a solvent mineral oils having a boiling point curve starting at a high temperature, for instance 300° C., a low freezing point, preferably not above -20° C., and the highest possible 95 flash point. The bitumen to be dissolved in an oil of this kind should be such as to dissolve therein without producing any slimy residue.

In producing a solution which is well 100 adapted for sealing purposes as hereinbefore described, I may for instance dissolve twenty parts mineral oil pitch in eighty parts mineral oil having a specific gravity

of 0.915, a flash point of 153° C. and a freezing point below —22° C., this oil, when subjected to fractional distillation resulting in the following fractions:

| ° C.       | Per cent |
|------------|----------|
| 300-310    | 10       |
| 310-320    | 11       |
| 320-330    | 14½      |
| 330-340    | 13.6     |
| 10 340-350 | 10.1     |
| 350-360    | 11.1     |
| Residue    | 29.7     |

15 A solution of the kind mentioned above, when used for sealing the disc in a gasometer, will not suffer any variation of its low freezing point; it will not thicken and will stand the test mentioned above (passage of air at 60° C.). With water the 20 solution will not form an emulsion, the water being separated out after a short rest, so as to be easily removed from time to time by hand or by mechanical means. In consequence thereof there does not exist any 25 danger of corrosion, the new product on the contrary forming an excellent means for preventing rusting of the walls. The term "mineral oil" used in the appended claims is intended to include ordinary mineral oil, 30 brown coal tar oil and low temperature coal tar oil, all containing a large percentage of paraffines.

I wish it to be understood that I do not desire to be limited to the exact substances, 35 proportions and temperatures above de-

scribed, for obvious modifications will occur to a person skilled in the art.

I claim:

1. As a new composition of matter for the sealing of gasometer discs, a solution of 40 mineral bitumen in a mineral oil, said oil starting to boil at about 300° C., having a freezing point not above —20° and a flash point not below 150° C.

2. As a new composition of matter for 45 the sealing of gasometer discs, a solution of mineral oil pitch in a mineral oil, said oil starting boiling at about 300° C. having a freezing point not above —20° C. and a flash point not below 150° C. 50

3. As a new composition of matter for the sealing of gasometer discs, a solution of 20 parts mineral oil pitch in 80 parts mineral oil having a specific gravity of about 0.915, a flash point of 153° C. and a freezing point below —22° C. 55

4. A sealing liquid for dry gasometers of the movable disc type comprising a mineral bituminous material and an oil vehicle therefor, said oil vehicle being an oil 60 consisting largely of aliphatic hydrocarbons, containing no substantial fractions boiling below 300° C., said oil having a flash point not substantially below 153° C., having a freezing point substantially below 65 that of water, and being substantially unaffected by illuminating gases.

In testimony whereof I affix my signature.

ROBERT MEZGER.